

# United States Patent [19]

Satoh et al.

[11] Patent Number: 4,708,748

[45] Date of Patent: Nov. 24, 1987

[54] **METHOD OF MAKING COLD ROLLED DUAL-PHASE STRUCTURE STEEL SHEET HAVING AN EXCELLENT DEEP DRAWABILITY**

[75] Inventors: **Susumu Satoh; Hideo Suzuki; Takashi Obara; Minoru Nishida; Osamu Hashimoto**, all of Chiba, Japan

[73] Assignee: **Kawasaki Steel Corporation**, Kobe, Japan

[21] Appl. No.: **881,915**

[22] Filed: **Jul. 3, 1986**

## Related U.S. Application Data

[60] Division of Ser. No. 790,641, Oct. 23, 1985, Pat. No. 4,615,749, which is a continuation of Ser. No. 591,406, Mar. 20, 1984, abandoned.

## Foreign Application Priority Data

Feb. 18, 1984 [JP] Japan ..... 59-27995

[51] Int. Cl. <sup>4</sup> ..... **C21D 8/04**

[52] U.S. Cl. ..... **148/2; 148/12 C; 148/12 F**

[58] Field of Search ..... **148/12 C, 12 D, 12 F, 148/12.4, 330; 148/2**

## References Cited

### U.S. PATENT DOCUMENTS

4,410,372 10/1983 Takahashi et al. ..... 148/12.4  
4,551,182 11/1985 Akisue et al. ..... 148/12 C

### FOREIGN PATENT DOCUMENTS

0085720 2/1983 European Pat. Off. ..... 148/12 C

5747828 3/1982 Japan ..... 148/12 F  
5852440 3/1983 Japan ..... 148/12 C  
5852430 3/1983 Japan ..... 148/12 F  
60197846 10/1985 Japan ..... 148/12 C  
2107226 4/1983 United Kingdom ..... 148/12 C

Primary Examiner—L. Dewayne Rutledge

Assistant Examiner—Deborah Yee

Attorney, Agent, or Firm—Balogh, Osann, Kramer, Dvorak, Genova & Traub

## ABSTRACT

A cold rolled dual-phase structure steel sheet having an excellent deep drawability is disclosed, which consists of ferrite phase and low temperature transformation product phase and comprises 0.001–0.008 wt % of C, not more than 1.0 wt % of Si, 0.05–1.8 wt % of Mn, not more than 0.15 wt % of P, 0.01–0.10 wt % of Al, 0.002–0.050 wt % of Nb and 0.0005–0.0050 wt % of B provided that the value of Nb(%) + 10B(%) is in a range of 0.010–0.080%, and, if necessary, 0.05–1.00 wt % of Cr and the balance being substantially Fe with inevitable impurities. This steel sheet is manufactured by hot and cold rolling a steel slab with the above chemical composition and continuously annealing the resulting steel sheet in such a manner that the steel sheet is heated and soaked at a temperature from  $\alpha \rightarrow \gamma$  transformation point to 1,000° C. and then cooled at an average cooling rate of not less than 0.5° C./sec but less than 20° C./sec in a temperature range of from the soaking temperature to 750° C., and subsequently at an average cooling rate of not less than 20° C./sec in a temperature range of from 750° C. to not more than 300° C.

3 Claims, 3 Drawing Figures



FIG. 1



FIG. 2



FIG. 3



**METHOD OF MAKING COLD ROLLED  
DUAL-PHASE STRUCTURE STEEL SHEET  
HAVING AN EXCELLENT DEEP DRAWABILITY**

This is a division of application Ser. No. 790,641, filed Oct. 23, 1985, now U.S. Pat. No. 4,615,749, which is a continuation of U.S. Ser. No. 591,406, filed Mar. 20, 1984, now abandoned.

**BACKGROUND OF THE INVENTION**

1. Field of the Invention

This invention relates to a cold rolled steel sheet suitable for use in, for example, automobile panels and the like requiring an excellent press formability. More particularly, the invention relates to an improvement in the properties of the above steel sheet through combined addition of Nb and B.

2. Description of the Prior Art

The cold rolled steel sheets for use in the above applications are required to have the following material characteristics:

(1) Deep Drawability: The deep drawability is evaluated by a Lankford value ( $r$ -value). The  $r$ -value of not less than 2.0 is required in case of deeper drawing.

(2) High ductility: A low yield strength (YS) and a high elongation (El) are required in order to achieve this characteristic.

(3) Non-aging property at room temperature: This means that the material is not deteriorated by the age hardening even when it is stored at room temperature for a long period of time.

(4) Resistance to denting: This means that the steel sheet after the press forming does not dent under a light load and is required to have a high yield strength of the steel sheet after the press forming.

Since the value YS is required to be low in the press forming, it is generally difficult to simultaneously realize both the press formability and the resistance to denting. However, it is possible to satisfy such conflicting properties in case of steel sheets having a property that it is hardened by the heating treatment (for instance, baked-on finish) subsequent to the press forming (hereinafter referred to as BH property).

The conventionally known cold rolled steel sheets for press forming are classified as follows:

(1) Steel sheets obtained by box annealing of low carbon aluminum-killed steel: This steel sheet is excellent in the deep drawability, ductility, and non-aging property at room temperature, but has almost no baking hardenability and also the resulting press formed parts are poor in the resistance to denting. Further, since the low carbon aluminum-killed steel is used as a raw material, it is difficult to secure the above-enumerated properties thereof by the continuous annealing method which is considered to be advantageous from the standpoints of the productivity and the homogeneity of the product.

(2) Steel sheets obtained by adding Nb or Ti to an extremely low carbon steel: This steel sheet exhibits excellent deep drawability and ductility even by the continuous annealing as in the case with the box annealing, and has the non-aging property at room temperature. Particularly, it has an extremely deep drawability because the  $r$ -value is not less than 1.8. However, it is not easy to provide the BH property likewise the case (1), so that the press formed part is poor in the resistance to denting.

(3) Dual-phase structure steel sheets in which ferrite and martensite phase are made coexistent by adding alloying elements such as Si, Mn, Cr, etc. to low carbon aluminum-killed steel and controlling the cooling rate after the continuous annealing. This steel sheet has the merit that because it has a lower yield strength as compared with the conventional steel sheet, it is excellent in the bulging property and is easy to gain a high strength. Further, it has a non-aging property at room temperature and a high BH property. However, it is poor in the drawability because the  $r$ -value is as low as about 1.0.

Although the methods of manufacturing cold rolled steel sheets having a dual-phase structure have hitherto been disclosed in U.S. Pat. Nos. 4,050,959, and 4,062,700, Japanese Patent Application Publication No. 53-39,368, Japanese Patent laid open Nos. 50-75,113 and 51-39,524 and so on, all of them do not relate to a method of manufacturing steel sheets with a high  $r$ -value, and are far behind the goal aiming at the invention.

**SUMMARY OF THE INVENTION**

It is, therefore, an object of the invention to provide a cold rolled steel sheet with a dual-phase structure possessing all of (1) high  $r$ -value, (2) high ductility, (3) non-aging property at room temperature, and (4) high BH property.

According to a first aspect of the invention, there is the provision of a cold rolled dual-phase structure steel sheet having an excellent deep drawability and consisting of ferrite phase and low temperature transformation product phase, which comprises 0.001-0.008% by weight of C, not more than 1.0% by weight of Si, 0.05-1.8% by weight of Mn, not more than 0.15% by weight of P, 0.01-0.10% by weight of Al, 0.002-0.050% by weight of Nb and 0.0005-0.0050% by weight of B provided that the value of  $Nb(\%) + 10B(\%)$  is in a range of 0.010-0.080%, and the balance being substantially Fe with inevitable impurities.

According to a second aspect of the invention, there is the provision of a method of manufacturing a cold rolled dual-phase structure steel sheet, comprising the steps of:

hot and cold rolling a steel slab with a composition containing 0.001-0.008% by weight of C, not more than 1.0% by weight of Si, 0.05-1.8% by weight of Mn, not more than 0.15% by weight of P, 0.01-0.10% by weight of Al, and 0.002-0.050% by weight of Nb and 0.0005-0.0050% by weight of B provided that the value of  $Nb(\%) + 10B(\%)$  is in a range of 0.010-0.080% by weight; and

continuously annealing the resulting steel sheet in such a manner that the steel sheet is heated and soaked at a temperature from  $\alpha \rightarrow \gamma$  transformation point to 1,000° C. and then cooled at an average cooling rate of not less than 0.5° C./sec but less than 20° C./sec in a temperature range of from the soaking temperature to 750° C., and subsequently at an average cooling rate of not less than 20° C./sec in a temperature range of from 750° C. to not more than 300° C.

According to a third aspect of the invention, there is the provision of a cold rolled dual-phase structure steel sheet having an excellent deep drawability and consisting of ferrite phase and low temperature transformation product phase, which comprises 0.001-0.008% by weight of C, not more than 1.0% by weight of Si, 0.05-1.8% by weight of Mn, not more than 0.15% by weight of P, 0.01-0.10% by weight of Al, 0.05-1.00%

by weight of Cr, 0.002–0.050% by weight of Nb and 0.0005–0.0050% by weight of B provided that the value of Nb(%) + 10B(%) is in a range of 0.010–0.080%, and the balance being substantially Fe with inevitable impurities.

According to a fourth aspect of the invention, there is the provision of a method of manufacturing a cold rolled dual-phase structure steel sheet, comprising the steps of:

hot and cold rolling a steel slab with a composition containing 0.001–0.008% by weight of C, not more than 1.0% by weight of Si, 0.05–1.8% by weight of Mn, not more than 0.15% by weight of P, 0.01–0.10% by weight of Al, 0.05–1.00% by weight of Cr, and 0.002–0.050% by weight of Nb and 0.0005–0.0050% by weight of B provided that the value Nb(%) + 10B(%) is in a range of 0.010–0.080%; and

continuously annealing the resulting steel sheet in such a manner that the steel sheet is heated and soaked at a temperature of from  $\alpha \rightarrow \gamma$  transformation point to 1,000° C. and then cooled at an average cooling rate of not less than 0.5° C./sec but less than 20° C./sec in a temperature range of from the soaking temperature to 750° C., and subsequently at an average cooling rate of not less than 20° C./sec in a temperature range of from 750° C. to not more than 300° C.

#### BRIEF DESCRIPTION OF THE DRAWINGS

The invention will be described in detail with reference to the accompanying drawing, wherein:

FIG. 1 is a graph showing the influence of Nb + 10B as a parameter upon YEL, YS and  $\bar{r}$ -value;

FIG. 2 is a graph showing the influence of the cooling rate from 750° C. of the continuous annealing heat cycle upon YEL, YR and  $\bar{r}$ -value; and

FIG. 3 is a graph showing the influence of the rapid cooling start temperature upon YEL, YS, TS, El and  $\bar{r}$ -value.

#### DETAILED DESCRIPTION OF THE INVENTION

First, the invention will be described from the studies based upon which the invention has been accomplished.

FIG. 1 shows the yield point elongation (YEL), yield strength (YS) and Lankford value ( $\bar{r}$ -value) of a cold rolled steel sheet obtained by hot rolling-cold rolling-continuous annealing of a steel slab with a composition containing C=0.004%, Mn=0.3%, N=0.004%, Al=0.05% and variable amounts of Nb and B.

The continuous annealing was carried out in such a heat cycle that the resulting steel sheet was heated to 910° C., soaked at the same temperature for 20 seconds, and was cooled at an average cooling rate of 3.0° C./sec at a temperature range of from the soaking temperature to 750° C. and at an average cooling rate of 27° C./sec at a temperature range of not more than 750° C. The measured values of the above properties were obtained with respect to a JIS No. 5 test piece of the aforementioned steel sheet without skin pass rolling.

As understood from FIG. 1, the non-aging property at room temperature is obtained only in the steel sheet containing both Nb and B and having YEL of not more than 1%.

Further, it has been confirmed that the structure of the steel sheet has a dual-phase structure consisting of a ferrite phase and a low temperature transformation product phase having a high dislocation density (which

is different from martensite phase of the conventional dual-phase structure steel sheet).

As shown in FIG. 1, the combined addition amount of Nb and B can be well related by a parameter of Nb(%) + 10B(%) to the properties of the steel sheet. When the value of Nb(%) + 10B(%) is less than 0.010%, the value of YEL is too high and no dual-phase structure is obtained, and the  $\bar{r}$ -value is low. On the other hand, when the value of Nb(%) + 10B(%) exceeds 0.080%, the value of YS largely increases and the  $\bar{r}$ -value drops.

As apparent from FIG. 1, a high  $\bar{r}$ -value, a low YS, and non-aging property at room temperature (a low YEL) are first satisfied by setting the parameter value of Nb(%) + 10B(%) in a range of 0.010–0.080%. Further, it was found that the steel sheet containing both Nb and B after the continuous annealing develops a property of largely increasing the yield strength (BH property) by applying a preliminary strain corresponding to a pressing force and subjecting to a heat treatment corresponding to a baked-on finish.

With respect to three kinds of small size steel ingots obtained by combining adding Cr, Nb and/or B to an extremely low carbon aluminum-killed steel containing C=0.005%, Mn=0.3% and Al=0.05% as base ingredients (Steel ingot X: Cr-Nb-B, Steel ingot Y: Nb-B, Steel ingot Z: Cr-B), FIG. 2 shows the relation of the average cooling rate in a temperature range of from 750° C. to room temperature at the time of annealing to the yield point elongation (YEL), the ratio of yield strength to tensile strength (YR) and the  $\bar{r}$ -value when the steel ingot is subjected to hot rolling-cold rolling-recrystallization annealing in laboratory. In this case, the soaking temperature was 900° C., and the cooling rate in a temperature range of from the soaking temperature to 750° C. was 5° C./sec. The values of the above properties were measured with respect to a JIS No. 5 test piece of the steel sheet without skin pass rolling.

In the Cr-B containing steel, the non-aging property at room temperature is not obtained because of the high YEL irrespective of the cooling rate, and the ductility is poor because the  $\bar{r}$ -value is low and YR is high.

On the other hand, the Nb-B containing steel can be imparted with the non-aging property at room temperature by controlling the cooling rate in the temperature range of from 750° C. to room temperature at not less than 20° C./sec, but YR is about 55% at this cooling rate and the ductility is slightly poor. Particularly, the Cr-Nb-B containing steel satisfies all of high  $\bar{r}$ -value, high ductility, and non-aging property at room temperature. It has also been found that the latter steel sheet has a so-called high BH property of increasing the yield strength by applying a light preliminary strain to the sheet and subjecting to a heat treatment at 170° C., and further confirmed that the structure of this steel sheet has the dual-phase structure consisting of a ferrite phase having a low dislocation density and a low temperature transformation product phase having a high dislocation density (which is different from martensite phase of the conventional dual-phase structure steel sheet).

The reasons why the composition of the steel sheet according to the invention is limited to the above ranges is as follows:

C: If C content exceeds 0.008%, the  $\bar{r}$ -value conspicuously drops. If it is less than 0.001%, a high BH property cannot be obtained. Thus, the C content of carbon is restricted to a range of 0.001–0.008%, preferably 0.002–0.004%.

Si, P: Si, and P are elements effective for obtaining the necessary strength level. If P is more than 0.15% and Si is more than 1%, the  $\bar{r}$ -value largely drops. Therefore, P is restricted to not more than 0.15% and Si is restricted to not more than 1.0%.

Mn: Mn is necessary to be not less than 0.05% for preventing red shortness. If it exceeds 1.8%, the  $\bar{r}$ -value largely drops. Therefore, Mn is restricted to a range of 0.05–1.8%, preferably 0.1–0.9%.

Al: Al is effective for reducing the oxygen content of the steel and precipitation-fixing N in the form of AlN. For this purpose, Al content should be not less than 0.01%. If Al content exceeds 0.10%, the non-metallic inclusion rapidly increases and the ductility is deteriorated. Thus, Al is restricted to a range of 0.01–0.10%.

Nb, B: These two alloying elements are particularly important in the invention, and the simultaneous addition of both the elements is indispensable therefor. If Nb is less than 0.002%, B is less than 0.0005%, and the value of Nb(%) + 10B(%) is less than 0.010%, no dual-phase structure steel sheet can be obtained. While, if Nb is more than 0.050%, B is more than 0.0050%, and the value of Nb(%) + 10B(%) is more than 0.080%, not only their addition effects are saturated, but also the ductility and  $\bar{r}$ -value are largely deteriorated. Therefore, according to the invention, it is essential that Nb is in a range of 0.002–0.050%, B is in a range of 0.0005–0.0050%, and the value of Nb(%) + 10B(%) is in a range of 0.010–0.080%. Moreover, the mechanism on the effect by the simultaneous addition of Nb and B is not yet clear. Although B is known to improve the hardenability of steel products, as shown in FIG. 1, low temperature transformation product phase is not formed by adding only B to the extremely low carbon aluminum-killed steel. Further, B is generally known to be an element of deteriorating the deep drawability ( $\bar{r}$ -value) of the cold rolled steel sheet, but according to the invention, an extremely high  $\bar{r}$ -value is attained in the steel sheet despite that it contains B.

That is, the effect by the simultaneous addition of Nb and B according to the invention has not been made public and is utterly novel.

According to the third aspect of the invention, the simultaneous addition of Cr, Nb and B is particularly important and indispensable.

Cr is particularly effective for obtaining a high  $\bar{r}$ -value and a low YR, i.e. a high ductility. If Cr content is less than 0.05%, the addition effect is not obtained, while if it exceeds 1.00%, not only the addition effect is saturated, but also the effect on the properties, particularly ductility is adversely affected. Therefore, the Cr content is limited to a range of 0.05–1.00%.

In the steel making, the extremely low carbon steel is most preferably melted by the combination of a bottom-blown converter and an RH degassing device.

The steel slab may be manufactured by either of blooming or continuous casting.

The hot rolling may be made by the conventional reheating system or direct hot-rolling method. Alternatively, a thin steel sheet of not more than 100 mm in thickness may be directly obtained from molten steel and subjected to hot rolling.

The optimum finishing temperature in the hot rolling is 950°–700° C.

Although the cooling means, the coiling temperature and so on of the hot rolled steel sheet are not so important according to the invention, the coiling temperature of not more than 600° C. is preferable from the standpoint of pickling.

The draft in the cold rolling is preferably not less than 50% in order to obtain a high  $\bar{r}$ -value.

The heating rate in the continuous annealing is not so important, but it is preferably not less than 10° C./sec from the standpoint of the productivity. The soaking temperature is preferably in a range of from  $\alpha \rightarrow \gamma$  transformation temperature to 1,000° C. The optimum range is 850°–950° C.

The cooling step after the soaking is important for obtaining the intended properties.

That is, it is necessary that the soaked sheet is subjected to a slow cooling from the soaking temperature to 750° C. at a cooling rate of 0.5°–20° C./sec and then cooled from 750° C. to not more than 300° C. at a cooling rate of not less than 20° C./sec. This will be described based on the experimental data below.

FIG. 3 shows the relation of the rapid cooling start temperature at the time of the annealing to the yield point elongation (YEl), yield strength (YS), tensile strength (TS), total elongation (El) and  $\bar{r}$ -value when a steel sheet containing 0.004% of C, 0.50% of Mn, 0.02% of P, 0.056% of Al, 0.015% of Nb and 0.0026% of B was subjected to hot rolling-cold rolling-recrystallization annealing. In this case, the soaking temperature was 900° C., the cooling rate up to the rapid cooling start temperature was 2° C./sec and the rapid cooling rate was 30° C./sec. The values of the above properties were measured with respect to a JIS No. 5 test piece of the steel sheet without skin pass rolling.

When the rapid cooling starts immediately from the soaking temperature, YEl becomes not more than 1% and the non-aging property at room temperature is attained but the yield strength becomes rather higher with respect to the tensile strength level and the elongation is low. On the contrary, when slow cooling is performed from the soaking temperature to 750° C., the reduction of YS and the increase of El are conspicuous. However, if slow cooling is performed down to 750° C., YEl abruptly increases.

It is understood from the above that the cooling step after the soaking in the continuous annealing is important for obtaining the desirable cold rolled steel sheet.

After the annealing, the steel sheet may be subjected to skin pass rolling for the purpose of correcting the profile thereof. In this case, the draft of the skin pass rolling is sufficient to be not more than 2% because the yield point elongation (YEl) is low.

On the other hand, the steel sheet according to the invention may be subjected to a surface treatment such as galvanization or the like without troubles. Particularly, the steel sheet according to the invention is suitable for the production of the surface treated steel sheet by hot dipping in an inline annealing system (including an alloying treatment).

Eight steel slabs were obtained by continuously casting steels A–H each having a chemical composition as shown in the following Table 1 after the treatment through the bottom-blown converter and RH-degassing device.

TABLE 1

| Steel | C     | Si   | Mn   | P     | S    | Al   | N      | Nb    | B      | Nb + 10B |
|-------|-------|------|------|-------|------|------|--------|-------|--------|----------|
| A*    | 0.005 | 0.02 | 0.30 | 0.014 | 0.01 | 0.05 | 0.0025 | 0.002 | 0.0002 | 0.004    |

TABLE 1-continued

| Steel | C     | Si   | Mn   | P     | S    | Al   | N      | Nb    | B      | Nb + 10B |
|-------|-------|------|------|-------|------|------|--------|-------|--------|----------|
| B     | 0.003 | 0.01 | 0.15 | 0.040 | 0.01 | 0.03 | 0.0036 | 0.011 | 0.0015 | 0.026    |
| C     | 0.004 | 0.02 | 0.60 | 0.015 | 0.01 | 0.07 | 0.0018 | 0.027 | 0.0030 | 0.057    |
| D*    | 0.007 | 0.02 | 0.30 | 0.020 | 0.01 | 0.06 | 0.0025 | 0.045 | 0.0062 | 0.107    |
| E*    | 0.010 | 0.01 | 0.32 | 0.016 | 0.01 | 0.04 | 0.0042 | 0.022 | 0.0026 | 0.048    |
| F     | 0.004 | 0.01 | 0.80 | 0.016 | 0.01 | 0.03 | 0.0016 | 0.018 | 0.0022 | 0.040    |
| G*    | 0.005 | 0.01 | 1.92 | 0.015 | 0.01 | 0.04 | 0.0033 | 0.020 | 0.0030 | 0.050    |
| H     | 0.004 | 0.02 | 0.51 | 0.81  | 0.01 | 0.04 | 0.0031 | 0.008 | 0.0025 | 0.033    |

\*Comparative Example

Each steel slab was soaked at 1,200° C., hot rolled at a finishing temperature of 860°–900° C. and at a coiling temperature of 500°–600° C. to obtain a steel sheet of 3.2 mm in thickness. After the pickling, it was cold rolled to be 0.8 mm in thickness and then subjected to a continuous annealing under such conditions that the soaking temperature is 910° C., the average cooling rate in a temperature range of from 910° C. to 750° C. is 3.2° C./sec, and the average cooling rate in a temperature range of from 750° C. to 250° C. is 40° C./sec, whereby there was obtained a cold rolled steel sheet having properties as shown in the following Table 2.

TABLE 2

| Steel | YEI<br>(%) | YS<br>(kg/mm <sup>2</sup> ) |                             | TS<br>(kg/mm <sup>2</sup> ) |                             | ΔYS<br>(kg/mm <sup>2</sup> ) | BH<br>(kg/mm <sup>2</sup> ) |     |
|-------|------------|-----------------------------|-----------------------------|-----------------------------|-----------------------------|------------------------------|-----------------------------|-----|
|       |            | YEI<br>(%)                  | TS<br>(kg/mm <sup>2</sup> ) | YEI<br>(%)                  | TS<br>(kg/mm <sup>2</sup> ) |                              |                             |     |
| A*    | 5.6        | 25                          | 32                          | 78.1                        | 44                          | 1.73                         | 4.2                         | 6.3 |
| B     | 0.3        | 17                          | 31                          | 54.8                        | 50                          | 2.34                         | 0.4                         | 4.8 |
| C     | 0.1        | 20                          | 36                          | 55.6                        | 45                          | 2.12                         | 0.6                         | 5.2 |
| D*    | 0.5        | 25                          | 34                          | 73.5                        | 39                          | 1.40                         | 0.7                         | 4.5 |
| E*    | 4.1        | 27                          | 34                          | 79.4                        | 38                          | 1.53                         | 3.5                         | 6.2 |
| F     | 0.4        | 23                          | 38                          | 60.5                        | 41                          | 2.02                         | 0.6                         | 5.5 |
| G*    | 0.2        | 28                          | 44                          | 63.6                        | 31                          | 1.26                         | 0.4                         | 5.1 |
| H     | 0          | 24                          | 40                          | 60.0                        | 38                          | 2.14                         | 0.3                         | 4.5 |

\*Comparative Example

The tensile test was made with respect to a JIS No. 5 test piece of the steel sheet. In Table 2,  $\Delta$ YS is represented by the increased amount (kg/mm<sup>2</sup>) of YS after the aging treatment at 35° C. for 100 days, and BH is represented by the difference between the deformation stress produced in the application of preliminary strain under a 2% tension and deformation strain produced in the treatment corresponding to a bake-on finish at 170°

obtain a cold rolled steel sheet having properties as shown in the following Table 4.

TABLE 3

| Steel C | Average cooling rate<br>from 910° C. to 750° C.<br>(°C./sec) |     | Average cooling rate<br>from 750° C. to 280° C.<br>(°C./sec) |    |
|---------|--------------------------------------------------------------|-----|--------------------------------------------------------------|----|
|         | 1*                                                           | 2   | 3                                                            | 4* |
| 1*      | 0.3                                                          |     |                                                              | 41 |
| 2       |                                                              | 1.1 |                                                              | 34 |
| 3       |                                                              | 2.5 |                                                              | 33 |
| 4*      |                                                              | 2.0 |                                                              | 14 |
| 5       |                                                              | 15  |                                                              | 65 |
| 6*      |                                                              | 25  |                                                              | 40 |

\*Comparative Example

TABLE 4

| Steel C | YEI<br>(%) | YS<br>(kg/mm <sup>2</sup> ) |                             | TS<br>(kg/mm <sup>2</sup> ) |                             | ΔYS<br>(kg/mm <sup>2</sup> ) | BH<br>(kg/mm <sup>2</sup> ) |
|---------|------------|-----------------------------|-----------------------------|-----------------------------|-----------------------------|------------------------------|-----------------------------|
|         |            | YEI<br>(%)                  | TS<br>(kg/mm <sup>2</sup> ) | YEI<br>(%)                  | TS<br>(kg/mm <sup>2</sup> ) |                              |                             |
| 1*      | 4.1        | 24                          | 34                          | 45                          | 1.81                        | 3.2                          | 5.8                         |
| 2       | 0.5        | 19                          | 35                          | 46                          | 2.16                        | 0.6                          | 4.9                         |
| 3       | 0.1        | 20                          | 36                          | 45                          | 2.30                        | 0.6                          | 5.2                         |
| 4*      | 5.1        | 26                          | 33                          | 44                          | 1.91                        | 4.0                          | 3.5                         |
| 5       | 0          | 20                          | 37                          | 44                          | 2.07                        | 0.2                          | 6.0                         |
| 6*      | 1.1        | 24                          | 37                          | 36                          | 1.75                        | 1.5                          | 5.6                         |

\*Comparative Example

It is apparent from Table 4 that the steel sheet (2, 3 and 5) treated under the optimum conditions of the invention have the intended excellent properties.

Ten steel slabs were obtained by continuously casting steels I–R each having a chemical composition as shown in the following Table 5 after the treatment through the bottom-blown converter and RH-degassing device.

TABLE 5

| Steel | C     | Si   | Mn   | P    | S    | Al     | N      | Cr   | Nb    | B      | (wt %)   |
|-------|-------|------|------|------|------|--------|--------|------|-------|--------|----------|
|       |       |      |      |      |      |        |        |      |       |        | Nb + 10B |
| I*    | 0.005 | 0.01 | 0.50 | 0.01 | 0.01 | 0.045  | 0.0032 | 0.35 | 0.002 | 0.0002 | 0.004    |
| J     | 0.003 | 0.02 | 0.80 | 0.01 | 0.01 | 0.036  | 0.0025 | 0.36 | 0.010 | 0.0008 | 0.018    |
| K     | 0.004 | 0.01 | 0.15 | 0.10 | 0.01 | 0.025  | 0.0042 | 0.80 | 0.006 | 0.0030 | 0.036    |
| L     | 0.004 | 0.02 | 0.53 | 0.01 | 0.01 | 0.0205 | 0.0026 | 0.40 | 0.015 | 0.0025 | 0.040    |
| M     | 0.008 | 0.85 | 0.40 | 0.05 | 0.01 | 0.060  | 0.0025 | 0.10 | 0.015 | 0.0045 | 0.060    |
| N*    | 0.003 | 0.02 | 0.52 | 0.05 | 0.01 | 0.018  | 0.0022 | 0.52 | 0.048 | 0.0043 | 0.091    |
| O*    | 0.012 | 0.01 | 0.51 | 0.02 | 0.01 | 0.035  | 0.0026 | 0.40 | 0.020 | 0.0025 | 0.045    |
| P*    | 0.005 | 0.02 | 2.15 | 0.01 | 0.01 | 0.042  | 0.0042 | 0.50 | 0.019 | 0.0030 | 0.049    |
| Q*    | 0.004 | 0.01 | 0.56 | 0.01 | 0.01 | 0.028  | 0.0022 | 0.02 | 0.025 | 0.0020 | 0.045    |
| R*    | 0.004 | 0.0  | 0.15 | 0.02 | 0.01 | 0.033  | 0.0018 | 1.16 | 0.009 | 0.0025 | 0.034    |

\*Comparative Example

C. for 20 minutes. In the invention steels (B, C, F and H), the  $\bar{r}$ -value is not less than 2.0, and a high ductility, non-aging property at room temperature, and a high BH property are obtained. Moreover, examples C, H, and F are production examples of high strength cold rolled steel sheets having TS of not less than 35 kg/mm<sup>2</sup>.

On the other hand, the steel having the composition C of Table 1 was subjected to a continuous annealing under conditions shown in the following Table 3 to

60 65 a cold rolled steel sheet having properties as shown in the following Table 4.

Each steel slab was soaked at 1,200° C., hot rolled at a finishing temperature of 860°–900° C. and at a coiling temperature of 500°–600° C. to obtain a steel sheet of 3.2 mm in thickness. After the pickling, it was cold rolled to be 0.8 mm in thickness and then subjected to a continuous annealing under such conditions that the soaking temperature is 900° C., the average cooling rate in a temperature range of from 910° C. to 750° C. is 4.2° C./sec, and the average cooling rate in a temperature range of from 750° C. to 280° C. is 34° C./sec, whereby

there was obtained a cold rolled steel sheet having properties as shown in the following Table 6.

TABLE 6

| Steel | YEI (%) | YS (kg/mm <sup>2</sup> ) | TS (kg/mm <sup>2</sup> ) | YR (%) | EI (%) | $\bar{r}$ | $\Delta YS$ (kg/mm <sup>2</sup> ) | BH (kg/mm <sup>2</sup> ) |
|-------|---------|--------------------------|--------------------------|--------|--------|-----------|-----------------------------------|--------------------------|
| I*    | 6.5     | 27                       | 33                       | 82     | 40     | 1.4       | 4.5                               | 5.0                      |
| J     | 0.3     | 17.5                     | 38                       | 46     | 42     | 2.2       | 0.6                               | 5.2                      |
| K     | 0.2     | 19                       | 42                       | 45     | 39     | 2.1       | 0.3                               | 5.7                      |
| L     | 0       | 15                       | 33                       | 45     | 46     | 2.3       | 0.3                               | 4.3                      |
| M     | 0.5     | 21                       | 45                       | 46     | 36     | 2.0       | 0.5                               | 4.6                      |
| N*    | 0.1     | 25                       | 37                       | 68     | 32     | 1.5       | 0.4                               | 3.5                      |
| O*    | 3.5     | 27                       | 35                       | 77     | 29     | 1.3       | 3.1                               | 4.5                      |
| P*    | 0.6     | 31                       | 46                       | 67     | 25     | 1.2       | 0.5                               | 5.2                      |
| Q*    | 0.4     | 21                       | 37                       | 57     | 37     | 1.5       | 0.8                               | 4.5                      |
| R*    | 0.5     | 25                       | 36                       | 70     | 38     | 1.5       | 0.4                               | 3.8                      |

\*Comparative Example

The tensile test was made with respect to a JIS No. 5 test piece of the steel sheet. In Table 6,  $\Delta YS$  is represented by the increased amount (kg/mm<sup>2</sup>) of YS after the aging treatment at 35° C. for 100 days, and BH is represented by the difference between the deformation stress produced in the application of preliminary strain under a 2% tension and deformation strain produced in the treatment corresponding to a bake-on finish at 170° C. for 20 minutes. In the invention steels (J, K, L and M), a high  $\bar{r}$ -value, a high ductility, non-aging property at room temperature, and a high BH property are obtained.

On the other hand, the steel having the composition L of Table 5 was subjected to a continuous annealing under conditions shown in the following Table 7 to obtain a cold rolled steel sheet having properties as shown in the following Table 8.

TABLE 7

| Steel L | Average cooling rate from soaking temperature to 750° C. (°C./sec) | Average cooling rate from 750° C. to 280° C. (°C./sec) | Soaking temperature (°C.) |
|---------|--------------------------------------------------------------------|--------------------------------------------------------|---------------------------|
| 1*      | 1.2                                                                | 40                                                     | 770                       |
| 2*      | 0.3                                                                | 32                                                     | 880                       |
| 3       | 0.9                                                                | 41                                                     | 830                       |
| 4       | 3.2                                                                | 25                                                     | 960                       |
| 5*      | 23                                                                 | 31                                                     | 910                       |
| 6*      | 2.5                                                                | 15                                                     | 920                       |
| 7       | 2.7                                                                | 75                                                     | 890                       |
| 8*      | 1.8                                                                | 38                                                     | 1,040                     |

\*Comparative Example

TABLE 8

| Steel L | YEI (%) | YS (kg/mm <sup>2</sup> ) | TS (kg/mm <sup>2</sup> ) | YR (%) | EI (%) | $\bar{r}$ | $\Delta YS$ (kg/mm <sup>2</sup> ) | BH (kg/mm <sup>2</sup> ) |
|---------|---------|--------------------------|--------------------------|--------|--------|-----------|-----------------------------------|--------------------------|
| 1*      | 7.2     | 25                       | 34                       | 74     | 45     | 1.4       | 3.5                               | 6.1                      |
| 2*      | 2.1     | 24                       | 33                       | 73     | 45     | 1.7       | 2.4                               | 5.6                      |
| 3       | 0.1     | 15.5                     | 34                       | 46     | 45     | 2.1       | 0.5                               | 5.1                      |
| 4       | 0.4     | 15                       | 33                       | 45     | 47     | 2.3       | 0.2                               | 5.8                      |
| 5*      | 3.5     | 21                       | 37                       | 57     | 38     | 1.7       | 3.8                               | 5.2                      |
| 6*      | 6.5     | 26                       | 32                       | 81     | 43     | 1.8       | 4.2                               | 6.3                      |
| 7       | 0.2     | 15.5                     | 35                       | 44     | 43     | 2.0       | 0.5                               | 5.5                      |
| 8*      | 0.5     | 18                       | 34                       | 53     | 32     | 1.4       | 1.0                               | 4.5                      |

\*Comparative Example

It is seen apparent from Table 8 that the steel sheets (L-3, L-4 and L-7) treated under the optimum conditions according to the third aspect of the invention have the intended excellent properties.

According to the first and third aspects of the invention, it is possible to realize a deep drawability, a high ductility, and non-aging property at room temperature together with a sufficiently high resistance to denting under a low YS before press forming, in case of the cold

rolled steel sheets which are required to have an excellent press formability for use in automobile panels and so on, and also these steel sheets can advantageously be manufactured according to the second and fourth aspects of the invention.

What is claimed is:

1. A method of manufacturing a cold rolled dual-phase structure steel sheet to obtain a sheet having deep drawability ( $\bar{r}$ -value), comprising the steps of:

5 10 selecting a steel slab with a composition containing 0.001–0.008% by weight of C, not more than 1.0% by weight of Si, 0.05–1.8% by weight of Mn, not more than 0.15% by weight of P, 0.01–0.10% by weight of Al, and combining 0.002–0.050% by weight of Nb and 0.0005–0.0050% by weight of B provided that the combined value of  $Nb(\%) + 10B(\%)$  is in a range of 0.010–0.080% by weight, hot and cold rolling said steel slab to obtain a steel sheet; and

15 continuously annealing the said steel sheet in such a manner that the steel sheet is heated and soaked at a temperature from  $\alpha \rightarrow \gamma$  transformation point to 1,000° C. and then cooled at an average cooling rate of not less than 0.5° C./sec but less than 20° C./sec in a temperature range of from the soaking temperature to 750° C., and subsequently at an average cooling rate of not less than 20° C./sec in a temperature range of from 750° C. to not more than 300° C.

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 741

3. A method of manufacturing a cold rolled dual-phase structure steel sheet to obtain a sheet having deep drawability ( $\bar{r}$ -value), comprising the steps of:

smelting and casting to form a steel slab with a composition containing 0.001-0.008% by weight of C, not more than 1.0% by weight of Si, 0.05-1.8% by weight of Mn, not more than 0.15% by weight of P, 0.01-0.10% by weight of Al, and combining 0.002-0.050% by weight of Nb and 0.0005-0.0050% by weight of B provided that the combined value of Nb(%) + 10B(%) is in a range of

5

10

0.010-0.080% by weight, hot and cold rolling said steel slab to obtain a steel sheet; and continuously annealing the said steel sheet in such a manner that the steel sheet is heated and soaked at a temperature from  $\alpha \rightarrow \gamma$  transformation point to 1,000° C. and then cooled at an average cooling rate of not less than 0.5° C./sec but less than 20° C./sec in a temperature range of from the soaking temperature to 750° C., and subsequently at an average cooling rate of not less than 20° C./sec in a temperature range of from 750° C. to not more than 300° C.

\* \* \* \* \*

15

20

25

30

35

40

45

50

55

60

65